

Patented Nov. 30, 1926.

## UNITED STATES PATENT OFFICE.

SHINJIRO HORII, OF TOKYO, JAPAN.

## STENCIL SHEET.

No Drawing.

Application filed January 15, 1926. Serial No. 81,585.

My invention relates to the production of stencil sheets of the type commonly used for autographic and typewriting duplication, and consisting of a sheet of fibrous material, such as Japanese yoshino paper, coated or impregnated with a colloidal composition.

The object of the present invention is to produce an improved stencil sheet, which has a considerable resistance to atmospheric influences and produces sharp and uniform copy through the pressure of the stylus or the impact of the types of a typewriting machine, so that a great number of clear copies can be obtained from one original.

In the production of stencil sheets it has been proposed to use for coating the porous support, such as yoshino paper, a solution containing monopole soap, or soft soap, in small proportions in a coating composition including gelatine, Irish moss and a considerable proportion of glycerine.

According to the present invention, the composition comprises Funori and alkali soaps of solid fats, such as hardened oils, tallow or Japan wax together with glycerine. The alkali soaps of solid fats are much less soluble than those of liquid fatty oils and produce a gelatinous mass from their aqueous solution. This gelatinized soap solution when intimately mixed with Funori and glycerine produces a colloidal composition which forms a stable and durable coating specially suitable for stencil sheets. If desired, a small amount of agar-agar, or gelatine may be added to the above mixture for the purpose of improving the property

of the coating. The above mentioned coating composition may be added to the paper pulp in a mixing hollander during the paper making operation.

Funori is a seaweed (genus *Gloiopeletis J. Ag.*) indigenous to Japan, which makes a viscous colloidal solution of higher concentration than any other gelatinizing organic colloids, such as agar-agar, Irish moss, gelatine, etc. This property gives it the special advantages as an ingredient of the colloidal composition for the stencil paper, making the coating operation very easy and resulting in a moderately soft and a very superior coating.

The proportions of the ingredients of the composition may vary according to circumstances. The following may be cited as an example:

|                        | Parts in weight. |
|------------------------|------------------|
| Funori                 | 10               |
| Agar-agar              | 2                |
| Soda soap of Japan wax | 10               |
| Glycerine              | 20               |
| Water                  | 500              |

## What I claim is:

1. A stencil sheet comprising a base of fibrous material impregnated with a colloidal composition including Funori, an alkali soap of solid fats and glycerine.
2. A stencil sheet comprising a base of fibrous material impregnated with a colloidal composition including Funori, agar-agar, an alkali soap of solid fats and glycerine.

In testimony whereof I affix my signature.  
SHINJIRO HORII.